

## UNITED STATES PATENT OFFICE

2,339,252

## MANGANESE NICKEL ALLOY

Reginald S. Dean, Washington, D. C., and Clarence T. Anderson, Pittsburgh, Pa., assignors to Chicago Development Company, Chicago, Ill., a corporation of Illinois

No Drawing. Application November 6, 1939,  
Serial No. 303,007

2 Claims. (Cl. 148—32)

This invention relates to alloys of manganese and nickel. It relates to ductile alloys of manganese and nickel containing from 50 to 95% manganese, the remainder substantially nickel.

We have found that when alloys within this composition range are prepared with pure manganese, such as electrolytic manganese, they are highly ductile when rapidly cooled from temperatures approaching their melting points.

We have found that these alloys are susceptible to improvement by aging at elevated temperatures. The following table illustrates the hardness of the alloys of our invention when rapidly cooled, cold worked, aged at 450 degrees C. and aged at 550 degrees C.

| Composition |    | Hardness, Rockwell C |             |                 |                 |
|-------------|----|----------------------|-------------|-----------------|-----------------|
| Mn          | Ni | Rapidly cooled       | Cold worked | Aged at 450° C. | Aged at 550° C. |
| 60          | 40 | —4                   | +26         | +52             | 30              |
| 65          | 35 | —4                   | 27          | 49              | 25              |
| 70          | 30 | —11                  | 16          | 21              | 8               |
| 75          | 25 | —12                  | 14          | 14              | 6               |
| 80          | 20 | —20                  | 10          | 10              | 5               |
| 85          | 15 | —21                  | 6           | 6               | 20              |
| 90          | 10 | —22                  | 5           | 5               | 36              |

This table shows that alloys containing less than 70% manganese harden greatly when aged at 450 degrees C. after quenching. Alloys from 70% to 80% manganese show relatively little hardening at 450 degrees C. Alloys containing more than 80% manganese show no hardening at 450 degrees C., but harden at 550 degrees C.

The table illustrates results obtaining by aging after quenching and cold working. Similar results may be obtained by eliminating the cold working step, it being understood, of course, that the rates of hardening are somewhat affected by the cold working. These alloys are non-magnetic. Their electrical resistance is relatively high in the quenched state. Alloys containing less than approximately 70% manganese show a decrease of electrical resistance on aging, while alloys containing more than 80% manganese show an increase of electrical resistance on aging. This is illustrated by the following table:

| Composition |    | Electrical resistance $\times 10^{-6}$ ohms/cm. <sup>2</sup> |                 |                 |
|-------------|----|--------------------------------------------------------------|-----------------|-----------------|
| Mn          | Ni | Quenched and cold worked                                     | Aged at 450° C. | Aged at 700° C. |
| 60          | 40 | 185                                                          | 160             | 175             |
| 65          | 35 | 185                                                          | 163             | 172             |
| 70          | 30 | 171                                                          | 178             | 185             |
| 75          | 25 | 163                                                          | 166             | 178             |
| 80          | 20 | 149                                                          | 151             | 168             |
| 85          | 15 | 132                                                          | 135             | 712             |
| 90          | 10 | 113                                                          | 145             | 1,550           |

We have found that the temperature coefficient of these alloys passes through zero between 65 and 70% manganese. With more manganese than 70%, the temperature coefficient is positive, while with less manganese, the temperature coefficient is negative. The coefficient of expansion of these alloys passes through a maximum at approximately 70% manganese having a value of more than  $22.5 \times 10^{-4}$  cm./cm./deg. C. From this maximum it falls to approximately  $16 \times 10^{-4}$  cm.<sup>3</sup>/deg. C. at 50%, and to  $15 \times 10^{-4}$  cm.<sup>3</sup>/deg. C. at 90%.

The alloys containing more than 70% manganese may be obtained with high vibration damping capacity by suitable heat treatment. We have found that a suitable heat treatment is to quench from 900 degrees C. and age at 450 degrees C. Under these conditions, vibration damping capacity of greater than 2% can be obtained. This figure may be compared to a corresponding figure for certain steels which is less than .04%.

The tensile strength in the quenched and cold worked alloys follows the Rockwell hardness in a manner approximately similar to steel. The quenched and cold worked alloys are especially tough in the quenched condition. The elongation in this condition is more than 40% in two inches, with tensile strengths as high as 75,000 lbs. per sq. in. Alloys within the range given, containing less than 70% manganese, are tough in the aged and hardened states. Extreme hardness in alloys containing more than 70% manganese is accompanied by some brittleness, but not enough to prevent their being employed for many useful purposes.

What is claimed as new and desired to be protected by Letters Patent of the United States is:

1. A ductile alloy of manganese and nickel containing from 75% to 95% manganese, hardened by quenching from a temperature between 800 degrees C. and its melting point and aging at a temperature above 500 degrees C.

2. A ductile alloy of manganese and nickel containing from 75% to 95% of electrolytic manganese of high purity, said alloy being hardened by a heating, quenching, aging procedure.

REGINALD S. DEAN.  
CLARENCE T. ANDERSON.